



US005250405A

**United States Patent** [19]

Merkel et al.

[11] Patent Number: **5,250,405**[45] Date of Patent: **Oct. 5, 1993**

[54] **COLOR PHOTOGRAPHIC MATERIALS INCLUDING MAGENTA COUPLER, INHIBITOR-RELEASING COUPLER AND CARBONAMIDE COMPOUND, AND METHODS**

[75] Inventors: **Paul B. Merkel, Rochester; Stephen P. Singer, Spencerport, both of N.Y.**

[73] Assignee: **Eastman Kodak Company, Rochester, N.Y.**

[21] Appl. No.: **752,147**

[22] Filed: **Aug. 29, 1991**

[51] Int. Cl.<sup>5</sup> ..... **G03C 1/08; G03C 7/26; G03C 7/32**

[52] U.S. Cl. ..... **430/544; 430/546; 430/555; 430/377; 430/387**

[58] Field of Search ..... **430/546, 544, 555, 377, 430/387**

[56] **References Cited**

**U.S. PATENT DOCUMENTS**

4,171,975 10/1979 Kato ..... 430/554  
4,483,918 7/1984 Sakai et al. ..... 430/372  
4,585,728 6/1986 Furutachi et al. ..... 430/372  
4,857,449 1/1989 Ogawa et al. ..... 430/546  
4,894,318 1/1990 Arakawa ..... 430/548

5,051,346 9/1991 Fujiwhara ..... 430/546  
5,071,735 10/1991 Ichijima .

**FOREIGN PATENT DOCUMENTS**

3730557 7/1989 Fed. Rep. of Germany .  
2086597 5/1982 United Kingdom .  
2088075 6/1982 United Kingdom .

*Primary Examiner*—Charles L. Bowers, Jr.

*Assistant Examiner*—Geraldine Letscher  
*Attorney, Agent, or Firm*—Lowe, Price, LeBlanc & Becker

[57] **ABSTRACT**

Color photographic materials comprise a support bearing a silver halide emulsion and a coupler composition. The coupler composition comprises a two-equivalent pyrazolone magenta dye-forming coupler, a ballasted carbonamide compound, and a developer inhibitor-releasing coupler. The carbonamide compound reduces continued coupling of the pyrazolone magenta dye-forming coupler during the bleach step in a color photographic process without altering the advantageous properties provided by the combination of the two-equivalent pyrazolone magenta dye-forming coupler and the developer inhibitor-releasing coupler.

**18 Claims, No Drawings**

**COLOR PHOTOGRAPHIC MATERIALS  
INCLUDING MAGENTA COUPLER,  
INHIBITOR-RELEASING COUPLER AND  
CARBONAMIDE COMPOUND, AND METHODS**

**FIELD OF THE INVENTION**

The present invention relates to color photographic materials and methods employing two-equivalent pyrazolone magenta dye-forming couplers. More particularly, the invention relates to such materials and methods wherein the two-equivalent pyrazolone magenta dye-forming coupler is used in combination with a developer inhibitor-releasing coupler and a ballasted carbonamide compound.

**BACKGROUND OF THE INVENTION**

Color photographic materials employing two-equivalent pyrazolone magenta dye-forming couplers are known in the art as demonstrated, for example, by the Sakai et al U.S. Pat. No. 4,483,918, the Furutachi et al U.S. Pat. No. 4,585,728 and German Off. DE 3,730,557. Two-equivalent pyrazolone magenta couplers are advantageous for use in color photographic materials owing to their low cost, high efficiency, good activity, adjustable hue and suitability for use in processes without formaldehyde. However, one disadvantage associated with the two-equivalent pyrazolone magenta dye-forming couplers is that they have low pKa values. The pKa value is  $-\log K_a$ , wherein  $K_a$  is the acid dissociation constant. Since these couplers tend to have low pKa values, they may be significantly ionized when films or papers coated with them are placed in solutions of low pH, i.e., a pH of 5-6, or less. Thus, when photographic materials containing these low pKa couplers are used in a process which does not employ a stop bath between the development and bleach steps, non-image-wise dye formation occurs owing to coupling with developer that is carried over into the bleach solution and oxidized therein. This phenomenon, which is referred to as continued coupling, produces undesirable increases in background density (Dmin). Continued coupling also leads to unacceptable density variability in processed films owing to variations in bleach pH as the bleach solutions become "seasoned" by continued use. Accordingly, photographic films and papers containing low pKa couplers such as the two-equivalent pyrazolone couplers often exhibit continued coupling because the couplers are more highly ionized at low pH and thus readily react with oxidized developer in the low pH bleach solutions. Thus, there is a need to provide color photographic materials which contain two-equivalent pyrazolone magenta dye-forming couplers and which exhibit a reduction in the continued coupling phenomenon.

It is also well known in the color photographic art that couplers are used in combination with solvents which facilitate their incorporation in the photographic materials and/or improve one or more properties of the dyes formed from the couplers. For example, the Ogawa et al U.S. Pat. No. 4,857,449 discloses combinations of couplers and one or more high boiling organic solvents for use in color photographic materials. The Kato et al. U.S. Pat. No. 4,171,975 discloses aldehydebis type magenta couplers in combination with high boiling organic solvents and other additives.

It is also known to use magenta dye-forming couplers in combination with one or more image-modifying cou-

plers, particularly in color negative films. The image-modifying couplers release development inhibitors on reaction with oxidized developer to provide one or more functions such as gamma or curve shape control, sharpness enhancement, granularity reduction and color correction via interlayer effects. The image-modifying couplers include development inhibitor releasing (DIR) couplers from which inhibitor is released directly as a coupling-off group, and development inhibitor activated releasing (DIAR) couplers from which inhibitor is released as a coupling-off group after a timed delay which results from an additional chemical reaction step. Because the inhibitor releasing couplers are used in combination with the magenta dye-forming couplers to provide improved color images, it is important that any means for reducing the continued coupling phenomena of the magenta dye-forming couplers does not unfavorably alter the advantageous effects provided by the inhibitor releasing couplers.

**SUMMARY OF THE INVENTION**

Accordingly, it is an object of the present invention to provide improved color photographic materials and methods which employ two-equivalent pyrazolone magenta dye-forming couplers. It is a further object of the invention to provide color photographic materials and methods which employ two-equivalent pyrazolone magenta dye-forming couplers in combination with inhibitor-releasing couplers. It is an additional object of the invention to provide color photographic materials and methods which employ two-equivalent pyrazolone magenta dye-forming couplers in combination with inhibitor-releasing couplers and which exhibit a reduction in the continued coupling of the magenta dye-forming coupler during the bleach step of a color photographic process. It is a related object of the invention to provide such materials and methods exhibiting a reduction in the continued coupling phenomenon without disadvantageously effecting the improvements in color provided by the inhibitor-releasing couplers.

These and additional objects and advantages are provided by the materials and methods of the present invention. The color photographic materials of the invention comprise a support bearing a silver halide emulsion and a coupler composition comprising a two-equivalent pyrazolone magenta dye-forming coupler, a carbonamide compound, and a developer inhibitor-releasing coupler. The carbonamide compound acts as a solvent and reduces the continued coupling phenomena exhibited by the magenta dye-forming coupler. However, the carbonamide compound does not disadvantageously alter the improved effects provided by the inhibitor-releasing coupler. Thus, the color photographic materials according to the present invention provide images exhibiting gamma values similar to those obtained using conventional coupler solvents while substantially reducing undesirably high Dmin values and Dmin variability which are an indication of the continued coupling phenomenon. The ability of the carbonamide compound to reduce the continued coupling phenomenon without significantly changing the gamma values provided by a combination of the magenta coupler and the developer inhibitor-releasing coupler is surprising and unexpected, and advantageously provides improved color photographic materials and methods.

These and additional objects and advantages provided by the materials and methods of the present in-

vention will be more fully apparent in view of the following detailed description.

#### DETAILED DESCRIPTION

The color photographic materials according to the present invention comprise a support bearing a silver halide emulsion and a coupler composition. The coupler composition comprises a two-equivalent pyrazolone magenta dye-forming coupler, a carbonamide compound and a developer inhibitor-releasing coupler.

The coupler compositions employed in the present invention include a two-equivalent pyrazolone magenta dye-forming coupler. The two-equivalent pyrazolone magenta dye-forming coupler included in the coupler compositions of the present invention is of the formula:



wherein:

Ar is selected from the group consisting of unsubstituted aryl groups, substituted aryl groups and substituted pyridyl groups, the substituents being selected from the group consisting of halogen atoms and cyano, alkylsulfonyl, arylsulfonyl, sulfamoyl, sulfonamido, carbamoyl, carbonamido, alkoxy, acyloxy, aryloxy, alkoxy carbonyl, aryloxycarbonyl, ureido, nitro, alkyl and trifluoromethyl groups; Y is selected from the group consisting of anilino, acylamino and ureido groups and one of said groups substituted with one or more substituents selected from the group consisting of halogen atoms, and alkyl, aryl, alkoxy, aryloxy, carbonamido, carbamoyl, sulfonamido, sulfamoyl, alkylsulfoxyl, arylsulfoxyl, alkylsulfonyl, arylsulfonyl, alkoxy carbonyl, aryloxycarbonyl, acyl, acyloxy, ureido, imido, carbamate, heterocyclic, cyano, trifluoromethyl, alkylthio, nitro, carboxyl and hydroxyl groups, and groups which form a link to a polymeric chain, and wherein Y contains at least 6 carbon atoms; and

X is a coupling-off group selected from the group consisting of halogen atoms, and alkoxy, aryloxy, alkylthio, arylthio, acyloxy, sulfonamido, sulfonyloxy, carbonamido, arylazo, nitrogen-containing heterocyclic and imido groups.

Coupling-off groups are well known to those skilled in the photographic art. Generally, such groups determine the equivalency of the coupler and modify the reactivity of the coupler. Coupling-off groups can also advantageously effect the layer in which the coupler is coated or other layers in the photographic material by performing, after release from the coupler, such functions as development inhibition, bleach acceleration, color correction, development acceleration and the like. Representative coupling-off groups include, as noted above, halogens (for example, chloro), alkoxy, aryloxy, alkylthio, arylthio, acyloxy, sulfonamido, carbonamido, arylazo, nitrogen-containing heterocyclic groups such as pyrazolyl and imidazolyl, and imido groups such as succinimido and hydantoinyl groups. Except for the halogens, these groups may be substituted if desired. Coupling-off groups are described in further detail in: U.S. Pat. Nos. 2,355,169; 3,227,551;

3,432,521; 3,476,563; 3,617,291; 3,880,661; 4,052,212 and 4,134,766, and in British Patent References Nos. 1,466,788; 1,531,927; 1,533,039; 2,006,755A and 2,017,704A, the disclosures of which are incorporated herein by reference.

Other magenta couplers, specifically methylene bis-pyrazolone magenta dye-forming couplers are excluded from the compositions of the present invention.

10 As is well known in the photographic art, a dye-forming coupler should be nondiffusible when incorporated in a photographic element. That is, the coupler should be of such a molecular size and configuration that it will exhibit substantially no diffusion from the layer in which it is coated. To achieve this result, the total number of carbon atoms contained in Y should be at least 6. Preferably, Y contains from 6 to about 30 carbon atoms.

In a preferred embodiment of the two-equivalent 20 pyrazolone magenta dye-forming coupler of Formula (I), Ar is of the formula:



30 wherein R<sub>1</sub> is selected from the group consisting of halogen atoms and cyano, alkylsulfonyl, arylsulfonyl, sulfamoyl, sulfonamido, carbamoyl, carbonamido, ureido, alkoxy carbonyl, aryloxycarbonyl, acyloxy, alkoxy, aryloxy, nitro and trifluoromethyl groups.

35 If it is further preferred that Y is of the formula:



45 wherein

p is from zero to 2 and each R<sub>2</sub> is in a meta or para position with respect to R<sub>3</sub>;

50 each R<sub>2</sub> is individually selected from the group consisting of halogen atoms and alkyl, alkoxy, aryloxy, carbonamido, carbamoyl, sulfonamido, sulfamoyl, alkylsulfoxyl, arylsulfoxyl, alkylsulfonyl, arylsulfonyl, alkoxy carbonyl, aryloxycarbonyl, acyloxy, ureido, imido, carbamate, heterocyclic, cyano, nitro, acyl, trifluoromethyl, alkylthio and carboxyl groups, and;

55 R<sub>3</sub> is selected from the group consisting of hydrogen, halogen atoms and alkyl, alkoxy, aryloxy, alkylthio, carbonamido, carbamoyl, sulfonamido, sulfamoyl, alkylsulfonyl, arylsulfonyl, alkoxy carbonyl, acyloxy, acyl, cyano, nitro and trifluoromethyl groups. Preferably, R<sub>3</sub> is a chlorine atom or an alkoxy group.

In a further preferred embodiment of the magenta dye-forming coupler, the coupling-off group X is of the formula:



wherein  $R_4$  and  $R_5$  are individually selected from the group consisting of hydrogen, halogen atoms and alkyl,

(IV)

alkoxy, aryloxy, carbonamido, ureido, carbamate, sulfonamido, carbamoyl, sulfamoyl, acyloxy, alkoxy carbonyl, aryloxycarbonyl, amino and carboxyl groups; and wherein  $q$  is 0, 1 or 2 and  $R_5$  may be in the meta or para position with respect to the sulfur atom. Preferably,  $R_4$  has at least one carbon atom and the total number of carbon atoms in  $R_4$  and  $R_5$  combined is from 5 to about 25.

Examples of two-equivalent pyrazolone dye-forming magenta couplers suitable for use in the coupler compositions of the present invention include, but are not limited to, the following:



-continued



-continued



-continued



-continued



M16



M17



M18



M19



M20

-continued



Particularly preferred two-equivalent magenta dye-forming couplers for use in the present invention include those that have  $pK_a$  values of less than 10.0 when dispersed together with a coupler solvent.

The carbonamide compound included in the coupler compositions of the present invention is ballasted in order to minimize volatility, water solubility and diffusivity. The carbonamide compound acts as a solvent for the two-equivalent pyrazolone magenta dye-forming coupler and may be used in combination with one or more additional high-boiling cosolvents. It is preferred that the carbonamide compound included in the compositions of the present invention is of the formula:



(V) 40

wherein, R<sub>6</sub>, R<sub>7</sub> and R<sub>8</sub> are individually selected from the group consisting of (i) straight chain, branched and cyclic alkyl groups, straight chain and branched alkenyl groups and straight chain and branched alkylene groups, for example, forming bis compounds or rings; (ii) said alkyl groups, alkenyl groups and alkylene groups containing one or more substituents selected from the group consisting of alkoxy, aryloxy, aryl, alkoxycarbonyl, aryloxycarbonyl, and acyloxy groups and halogens; (iii) a phenyl group; and (iv) a phenyl group containing one or more substituents selected from the group consisting of alkyl, alkoxy, aryloxy, alkoxycarbonyl, aryloxycarbonyl and acyloxy groups and halogens; for example, chlorine and further wherein R<sub>6</sub>, R<sub>7</sub> and R<sub>8</sub> combined contain at least 12 carbon atoms. Preferably, R<sub>6</sub>, R<sub>7</sub> and R<sub>8</sub> combined contain from about 15 to about 30 carbon atoms in order to minimize volatility, water solubility and diffusivity. 45 50 55 60

In further preferred embodiments, at least one of  $R_6$ ,  $R_7$  and  $R_8$  is an alkyl group, and/or  $R_6$  and  $R_7$  or  $R_7$  and  $R_8$  form a ring, for example, a five-membered pyrrolidinone ring or a six-membered nitrogen containing ring.

Examples of the carbonamide compound included in 65 the coupler compositions of the invention include, but are not limited to, the following:

M21

M22



-continued



Developer inhibitor-releasing couplers useful for the practice of this invention are well known in the art and are described in U.S. Pat. Nos. 3,148,062; 3,227,554; 3,384,657; 3,379,529; 3,615,506; 3,617,291; 3,620,746; 3,701,783; 3,733,201; 4,049,455; 4,095,984; 4,248,962; 4,409,323; 4,477,563; 4,782,012 and 4,962,018 as well as in "Developer-Inhibitor-Releasing (DIR) Couplers for Color Photography," C. R. Barr, J. R. Thurtle and P. W. Vittum in *Photographic Science and Engineering*, Vol. 13, p. 174 (1969), incorporated herein by reference. Generally, the developer inhibitor-releasing (DIR) couplers include a coupler moiety and an inhibitor coupling-off moiety (IN). The inhibitor-releasing couplers may be of the time-delayed type (DIAR couplers)

which also include a timing moiety or chemical switch which produces a delayed release of inhibitor. In a preferred embodiment, the inhibitor moiety or group (IN) is selected from the following formulas (VI)-(X):



C17 40 wherein R<sub>9</sub> is selected from the group consisting of straight and branched alkyls of from 1 to about 8 carbon atoms, benzyl and phenyl groups and said groups containing at least one alkoxy substituent; R<sub>10</sub> is selected from R<sub>9</sub> and —SR<sub>9</sub>; R<sub>11</sub> is a straight or branched alkyl group of from 1 to about 5 carbon atoms and m is from 1 to 3; and R<sub>12</sub> is selected from the group consisting of hydrogen, halogens and alkoxy, phenyl and carbonamido groups, —COOR<sub>13</sub> and —NHCOR<sub>13</sub> wherein R<sub>13</sub> is selected from substituted and unsubstituted alkyl and aryl groups.

C18 45 C19 50 Although it is most preferred that the coupler moiety included in the developer inhibitor-releasing coupler is a magenta dye-forming coupler, small amounts of yellow or cyan dye-forming coupler moieties might also be included in the developer inhibitor-releasing couplers. For example, yellow dye-forming coupler moieties may be suitable for providing a low dye extinction coefficient or covering power. It may also be useful that the coupler moiety included in the developer inhibitor-releasing coupler forms colorless products or products that wash out of the photographic material during processing.

When the developer inhibitor-releasing coupler includes a timing group which produces the time-delayed release of the inhibitor group, it is preferred that the timing group or moiety is of one of the following formulas (XI) and (XII):



(XI)

5

10

-continued

(XII)



5

10

wherein IN is the inhibitor moiety, Z is selected from the group consisting of nitro, cyano, alkylsulfonyl and sulfonamido groups; n is 0 or 1; and R<sub>14</sub> is selected from the group consisting of substituted and unsubstituted alkyl and phenyl groups. The oxygen atom of each timing group is bonded to the coupling-off position of the respective coupler moiety of the DIAR.

Suitable developer inhibitor-releasing couplers for use in the present invention include, but are not limited to, the following:



-continued





The coupler compositions which are employed in the present invention include the two-equivalent pyrazolone magenta dye-forming coupler, the carbonamide compound and the developer inhibitor-releasing coupler in amounts suitable for providing a reduction in the continued coupling phenomenon and optimizing the color properties of the resulting image. Specifically, the carbonamide compound is included in an amount sufficient to reduce continued coupling of the pyrazolone magenta dye-forming coupler during the bleach step of a color photographic process. In a preferred embodiment, the pyrazolone magenta dye-forming coupler and the carbonamide compound are included in a weight ratio of from about 1:0.1 to about 1:10. The developer inhibitor-releasing coupler is included in an amount sufficient to advantageously alter the color properties of the resulting image. Preferably, the pyrazolone magenta dye-forming coupler and the developer inhibitor-releasing coupler are employed in a weight ratio of from about 1:0.01 to about 1:2.0, and more preferably from about 1:0.02 to about 1:0.5.

As noted above, the carbonamide compound acts as a solvent for the magenta dye-forming coupler. Additionally, one or more additional high-boiling organic compounds may also be employed as a co-solvent. Additional high-boiling coupler solvents that may be used in combination with the carbonamide compound include aryl phosphates, for example, tricresyl phosphate; alkyl phosphates, for example, trioctyl phosphate; mixed aryl alkyl phosphates; alkyl, aryl or mixed aryl alkyl phosphonates; phosphine oxides, for example, trioctyl phosphine oxide; aromatic esters, for example, dibutyl

phthalate; aliphatic esters, for example, dibutyl sebacate; alcohols, for example, 2-hexyl-1-decanol; phenols, for example, p-dodecylphenol; sulfonamides; and hydrocarbons, for example, dodecylbenzene.

The coupler compositions of this invention may also include conventional additives, including light stabilizers, such as phenols or chromanols, alkoxy benzenes, aniline derivatives and amines.

The photographic coupler compositions according to the present invention are employed in color photographic materials in a manner well known in the photographic art. For example, a supporting substrate may be coated with a silver halide emulsion and a coupler composition of the present invention comprising a two-equivalent magenta dye-forming pyrazolone coupler, a carbonamide compound and a DIR or DIAR coupler, with the carbonamide compound present in sufficient amounts to reduce the continued coupling of the two-equivalent pyrazolone coupler during bleaching. The photographic materials may then be imagewise exposed in a manner well known in the color photographic art, followed by development in a solution containing a primary aromatic amine developing agent. As further well known in the art, the primary aromatic amine developing agent is oxidized in an imagewise manner by reacting with exposed silver halide emulsion grains, and the oxidized developing agent reacts with the coupler to form dye.

In employing the materials and methods of the present invention, the coated photographic material containing the magenta dye-forming coupler can be re-

moved from the developer solution and placed directly in a bleaching solution without an intervening stop bath or wash step. The purpose of the bleaching solution is to reoxidize developed silver for subsequent fixation. However, the bleaching solution also oxidizes developing agent which is carried over in the absence of an intervening stop bath or wash. In conventional materials, the oxidized developer may react with coupler to produce non-imagewise dye (D<sub>min</sub>), i.e., the continued coupling phenomenon. The materials of this invention minimize the continued coupling.

The photographic materials of the present invention may be simple elements or multilayer, multicolor elements. Multicolor elements contain dye image-forming units sensitive to each of the three primary regions of the spectrum. Each unit can be comprised of a single emulsion layer or of multiple emulsion layers sensitive to a given region of the spectrum. The layers of the element, including the layers of the image-forming units, can be arranged in various orders as known in the art.

A typical multicolor photographic element comprises a support bearing a cyan dye image-forming unit comprising at least one red-sensitive silver halide emulsion layer having associated therewith at least one cyan dye-forming coupler, a magenta image-forming unit comprising at least one green-sensitive silver halide emulsion layer having associated therewith at least one magenta dye-forming coupler and a yellow dye image-forming unit comprising at least one blue-sensitive silver halide emulsion layer having associated therewith at least one yellow dye-forming coupler. The element may contain additional layers, such as filter layers, interleavers, overcoat layers, subbing layers, and the like. The element typically will have a total thickness (excluding the support) of from 5 to 30 microns.

In the following discussion of suitable materials for use in the elements of this invention, reference will be made to *Research Disclosure*, December 1978, Item 17643, and December 1989, Item No. 308119 published by Kenneth Mason Publications, Ltd., Dudley Annex, 12a North Street, Emsworth, Hampshire P010 7DQ, ENGLAND, the disclosures of which are incorporated herein by reference. This publication will be identified hereafter by the term "Research Disclosure." The elements of the invention can comprise emulsions and addenda described in these publications and publications referenced in these publications.

The silver halide emulsions employed in the elements of this invention can be comprised of silver bromide, silver chloride, silver iodide, silver chlorobromide, silver chloroiodide, silver bromoiodide, silver chlorobromoiodide or mixtures thereof. The emulsions can include silver halide grains of any conventional shape or size. Specifically, the emulsions can include coarse, medium or fine silver halide grains. High aspect ratio tabular grain emulsions are specifically contemplated, such as those disclosed by Wilgus et al U.S. Pat. No. 4,434,226, Daubendiek et al U.S. Pat. No. 4,424,310, Wey U.S. Pat. No. 4,399,215, Solberg et al U.S. Pat. No. 4,433,048, Mignot U.S. Pat. No. 4,386,145, Evans et al U.S. Pat. No. 4,504,570, Maskasky U.S. Pat. No. 4,400,463, Wey et al U.S. Pat. No. 4,414,306, Maskasky U.S. Pat. Nos. 4,435,501 and 4,4414,966 and Daubendiek et al U.S. Pat. Nos. 4,672,027 and 4,693,964, incorporated herein by reference. Also specifically contemplated are those silver bromoiodide grains with a higher molar proportion of iodide in the core of the grain than

in the periphery of the grain, such as those described in British Reference No. 1,027,146; Japanese Reference No. 54/48,521; U.S. Pat. Nos. 4,379,837; 4,444,877; 4,665,012; 4,686,178; 4,565,778; 4,728,602; 4,668,614 and 4,636,461; and in European Reference No. 264,954, incorporated by reference. The silver halide emulsions can be either monodisperse or polydisperse as precipitated. The grain size distribution of the emulsions can be controlled by silver halide grain separation techniques or by blending silver halide emulsions of differing grain sizes.

Sensitizing compounds, such as compounds of copper, thallium, lead, bismuth, cadmium and Group VIII noble metals, can be present during precipitation of the silver halide emulsion.

The emulsions can be surface-sensitive emulsions, i.e., emulsions that form latent images primarily on the surfaces of the silver halide grains, or internal latent image-forming emulsions, i.e., emulsions that form latent images predominantly in the interior of the silver halide grains. The emulsions can be negative-working emulsions, such as surface-sensitive emulsions or unfogged internal latent image-forming emulsions, or direct-positive emulsions of the unfogged, internal latent image-forming type, which are positive-working when development is conducted with uniform light exposure or in the presence of a nucleating agent.

The silver halide emulsions can be surface sensitized, and noble metal (e.g., gold), middle chalcogen (e.g., sulfur, selenium, or tellurium) and reduction sensitizers, employed individually or in combination, are specifically contemplated. Typical chemical sensitizers are listed in *Research Disclosure*, Item 17643, cited above, Section III.

The silver halide emulsions can be spectrally sensitized with dyes from a variety of classes, including the polymethine dye class, which includes the cyanines, merocyanines, complex cyanines and merocyanines (i.e., tri-, tetra-, and polynuclear cyanines and merocyanines), oxonols, hemioxonols, styryls, merostyryls, and streptocyanoanines. Illustrative spectral sensitizing dyes are disclosed in *Research Disclosure*, Item 17643, cited above, Section IV.

Suitable vehicles for the emulsion layers and other layers of elements of this invention are described in *Research Disclosure* Item 17643, Section IX and the publications cited therein.

In addition to the two-equivalent pyrazolone magenta couplers described herein, the elements of this invention can include additional couplers as described in *Research Disclosure* Section VII, paragraphs D, E, F and G and the publications cited therein. These additional couplers can be incorporated as described in *Research Disclosure* Section VII, paragraph C, and the publications cited therein. The coupler combinations of this invention can be used with colored masking couplers as described in U.S. Pat. No. 4,883,746 or with couplers that release bleach accelerators as described in European Patent Application No. 193,389.

The photographic elements of this invention can contain brighteners (*Research Disclosure* Section V), antifoggants and stabilizers (*Research Disclosure* Section VI), antistain agents and image dye stabilizers (*Research Disclosure* Section VII, paragraphs I and J), light absorbing and scattering materials (*Research Disclosure* Section VIII), hardeners (*Research Disclosure* X), coating aids (*Research Disclosure* Section XI), plasticizers and lubricants (*Research Disclosure* Section

XII), antistatic agents (Research Disclosure Section XIII), matting agents (Research Disclosure Sections XII and XVI) and development modifiers (Research Disclosure Section XXI).

The photographic elements can be coated on a variety of supports as described in Research Disclosure Section XVII and the references described therein.

The photographic elements of the invention can be exposed to actinic radiation, typically in the visible region of the spectrum, to form a latent image as described in Research Disclosure Section XVIII, and then processed to form a visible dye image as described in Research Disclosure Section XIX. Processing to form a visible dye image includes the step of contacting the element with a color developing agent to reduce developable silver halide and oxidize the color developing agent. Oxidized color developing agent in turn reacts with the coupler to yield a dye.

Preferred color developing agents are p-phenylenediamines. Especially preferred are 4-amino-3-methyl-N,N-diethylaniline hydrochloride, 4-amino-3-methyl-N-ethyl-N-β-(methanesulfonamido)-ethylaniline sulfate hydrate, 4-amino-3-methyl-N-ethyl-N-β-hydroxyethylaniline sulfate, 4-amino-3-β-(methanesulfonamido)ethyl-N,N-diethylaniline hydrochloride and 4-amino-N-ethyl-N,N-diethylaniline hydrochloride and 4-amino-N-ethyl-N-(2-methoxyethyl)-m-toluidine di-p-toluenesulfonic acid.

With negative-working silver halide, the processing step described above provides a negative image. The described elements are preferably processed in the known C-41 color process as described in, for example, the *British Journal of Photography Annual*, 1988, pages 196-198. To provide a positive (or reversal) image, the color development step can be preceded by development with a non-chromogenic developing agent to develop exposed silver halide, but not form dye, and then uniformly fogging the element to render unexposed silver halide developable. Alternatively, a direct positive emulsion can be employed to obtain a positive image.

Development is followed by the conventional steps of bleaching, fixing, or bleach-fixing, to remove silver or silver halide, washing, and drying.

The color photographic materials and methods of the present invention are demonstrated by the following examples, in which references are to parts by weight unless otherwise specified. References to comparative coupler solvents S1 and S2 refer, respectively, to mixed trityl phosphates and to dibutyl phthalate.

#### EXAMPLE 1

Preferred two-equivalent magenta dye-forming couplers for the practice of this invention include those that have pKa values of less than 10.0 when dispersed together with a coupler solvent. Potentiometric titrations were used to measure pKa values for some of the preferred couplers of the invention as aqueous dispersions. In these two-phase mixtures, the term pKa denotes the aqueous buffer pH at which half of the coupler in the oil phase is ionized or ion paired. Table I lists dispersion pKa values measured with 0.50M potassium counter ion.

TABLE I

| Coupler | Coupler Solvent | Coupler:Solvent Weight Ratio | pKa(0.5M K+) |
|---------|-----------------|------------------------------|--------------|
| M1      | S2              | 1:2                          | 8.5          |

TABLE I-continued

| Coupler | Coupler Solvent | Coupler:Solvent Weight Ratio | pKa(0.5M K+) |
|---------|-----------------|------------------------------|--------------|
| M7      | S2              | 1:2                          | 7.5          |
| M8      | S2              | 1:2                          | 7.9          |
| M20     | S2              | 1:2                          | 8.4          |
| M20     | C1              | 1:2                          | 8.9          |
| M3      | S1              | 1:1                          | 7.9          |
| M3      | C5              | 1:1                          | 8.2          |
| M4      | S1              | 1:1                          | 7.6          |
| M4      | C5              | 1:1                          | 8.0          |

#### EXAMPLE 2

15 Dispersions of couplers M1 and M2 were prepared in comparative coupler solvents S1 and S2 and in a carbonamide coupler solvent of this invention, C1. The weight ratio of coupler:solvent was 1:1. Dispersions were prepared by dissolving the coupler in a 1:3 mixture of coupler solvent plus cyclohexanone used as an auxiliary solvent. This mixture was then added to an aqueous solution of gelatin and ALKANOL XC surfactant. The two-phase mixture was passed through a colloid mill to disperse the coupler-containing oil phase in the aqueous phase in the form of small particles. The dispersion was then chilled, noodled and washed to remove the auxiliary cyclohexanone solvent. The resulting dispersions contained approximately 2% by weight of coupler and 6% by weight of gelatin.

20 30 The dispersions were coated on a transparent support at a coupler laydown of 0.54 mmole/m<sup>2</sup> together with a silver bromoiodide emulsion at a silver laydown of 1.08 g/m<sup>2</sup> in the following format:

35 2.69 g/m<sup>2</sup> Gelatin + 1.75 weight % BVSME Hardener  
0.54 mmole/m<sup>2</sup> Coupler (e.g. 0.50 g/m<sup>2</sup> of M1)  
Coupler Solvent @ equal weight to coupler  
3.77 g/m<sup>2</sup> Gelatin  
1.08 g/m<sup>2</sup> Silver as Silver Halide Emulsion  
40 Cellulose Acetate Butyrate Support

45 The BVSME hardener is of the formula (CH<sub>2</sub>=CH SO<sub>2</sub> CH<sub>2</sub>-<sub>2</sub>O. Coatings were then exposed and subjected to variants of the KODAK FLEXICOLOR (C-41) process described below. The C-41 process is described in

50 *British Journal of Photography Annual*, 1988, pp. 196-198, discussed above. A first set of films was subjected to the standard C-41 process with no stop bath between the development and bleach steps (process A).

55 A second set of films was also processed with out a stop bath but with the FLEXICOLOR bleach pH adjusted to 6.0 instead of the normal 5.25 (process B). This was intended to simulate behavior in a "seasoned" bleach with increased pH due to carry-over of base from the developer solution. A third set of films was processed with an acetic acid stop bath between the development and bleach steps to eliminate any continued coupling (process C).

| PROCESSING CONDITIONS |                                                                                                                                         |                            |
|-----------------------|-----------------------------------------------------------------------------------------------------------------------------------------|----------------------------|
| Step                  | Solution<br>(all at 100° F.)                                                                                                            | Time                       |
| 1                     | C-41 KF12 Developer                                                                                                                     | 3'15"                      |
| 2                     | A: Standard C-41 Bleach II;<br>or B: Bleach II Adjusted to pH = 6.0;<br>or C: Stop Bath, followed by<br>Standard C-41 Bleach II<br>Wash | 4'<br>4'<br>1'<br>4'<br>3' |
| 3                     |                                                                                                                                         |                            |

-continued

| PROCESSING CONDITIONS |                              |      |
|-----------------------|------------------------------|------|
| Step                  | Solution<br>(all at 100° F.) | Time |
| 4                     | C-41 Fix                     | 4'   |
| 5                     | Wash                         | 3'   |

The differences in Dmin values resulting from process A and process C or process B and process C are measures of the continued coupling at bleach pH values of 5.25 and 6.0, respectively. These differences are listed in Table II. Photographic gamma values, which serve as a measure of coupler activity, were obtained from plots of status M green density versus exposure for the various film samples subjected to process A. These gamma values are also listed in Table II.

TABLE II

| Coupler Coupler* | Delta Dmin Process A - C | Delta Dmin Process B - C | Delta Dmin Gamma |
|------------------|--------------------------|--------------------------|------------------|
| Solvent*         |                          |                          |                  |
| M1(1.0) S1(1.0)  | 0.04                     | 0.19                     | 2.10             |
| M1(1.0) S2(1.0)  | 0.10                     | 0.33                     | 2.41             |
| M1(1.0) C1(1.0)  | 0.01                     | 0.03                     | 1.84             |
| M2(1.0) S1(1.0)  | 0.05                     | 0.17                     | 1.92             |
| M2(1.0) S2(1.0)  | 0.09                     | 0.25                     | 2.04             |
| M2(1.0) C1(1.0)  | 0.00                     | 0.03                     | 2.29             |

\*Weight ratios are in parentheses.

As shown by the delta Dmin values in Table II, the carbonamide coupler solvent C1 is quite effective in reducing continued coupling in the absence of a stop bath. The reductions in Dmin without a stop bath are particularly large in the simulated seasoned (pH=6.0) bleach. Coupler activity remained high with carbonamide C1, as indicated by the gamma values in Table II.

## EXAMPLE 3

Dispersions of the pyrazolone magenta dye-forming coupler M2 were prepared in a mixture of S1 and aniline A1 (shown below) and in C5 by procedures similar to those described in Example 2.



An M2:S1:A1 weight ratio of 1:0.75:0.25 was used, and the M2:C5 weight ratio was 1:1. These dispersions were prepared without and with the DIR, D1, added at a M2:D1 weight ratio of 1:0.045. The dispersions were coated on a transparent support at a coupler laydown of 0.54 mmole/m<sup>2</sup> together with a silver bromoiodide emulsion at a silver laydown of 1.08 g/m<sup>2</sup> in a format similar to that of Example 2. Hardened coatings were exposed and processed using the procedures described in Example 2. The differences in Dmin values obtained with process B (Bleach pH=6.0, no stop bath) versus process C (Bleach pH=5.25, with stop bath), which are measures of continued coupling, are listed in Table III. Photographic gamma values obtained from plots of status M green density versus exposure are also listed in Table III.

| Imaging Coupler* | Coupler Solvent* | Aniline* | DIR Coupler* | Process B - C | Delta Dmin Gamma |
|------------------|------------------|----------|--------------|---------------|------------------|
| M2(1.0)          | S1(0.75)         | A1(0.25) | none         | 0.13          | 2.33             |
| M2(1.0)          | S1(0.75)         | A1(0.25) | D1(0.045)    | 0.14          | 1.69             |
| M2(1.0)          | C5(1.0)          | none     | none         | 0.06          | 3.04             |
| M2(1.0)          | C5(1.0)          | none     | D1(0.045)    | 0.10          | 2.07             |

\*Weight ratios are in parenthesis.

The data in Table III illustrates that, not only is carbonamide compound C5 more effective than an aniline compound A1 of the prior art in reducing continued coupling, but the carbonamide compositions yield higher gamma values, with and without the added DIR coupler D1.

## EXAMPLE 4

20 Dispersions of pyrazolone magenta dye-forming couplers M3 and M4 were prepared in combination with coupler solvents S1 and C5, with and without DIR coupler D1. The ratio of the pyrazolone coupler to the coupler solvent was 1:1. These dispersions were coated 25 on a transparent support at a coupler laydown of 0.54 mmole/m<sup>2</sup>, together with a silver bromoiodide emulsion at a silver laydown of 1.08 g/m<sup>2</sup>, as in Example 2. The differences in Dmin values obtained in process A (Bleach pH=5.25, no stop bath) and in process B (Bleach pH=6.0, no stop bath) and process C are listed 30 in Table IV. Larger differences are indicative of higher undesirable continued coupling. Photographic gamma values obtained from plots of status M green density versus exposure are also listed in Table IV.

TABLE IV

| Imaging Coupler* | Coupler Solvent* | DIR Coupler* | Process A - C | Process B - C | Delta Dmin Gamma |
|------------------|------------------|--------------|---------------|---------------|------------------|
| M3(1.0)          | S1(1.0)          | none         | 0.09          | 0.26          | 2.65             |
| M3(1.0)          | S1(1.0)          | D1(0.04)     | 0.11          | 0.30          | 1.52             |
| M3(1.0)          | C5(1.0)          | none         | 0.04          | 0.13          | 2.70             |
| M3(1.0)          | C5(1.0)          | D1(0.04)     | 0.05          | 0.13          | 1.60             |
| M4(1.0)          | S1(1.0)          | none         | 0.23          | 0.48          | 3.31             |
| M4(1.0)          | S1(1.0)          | D1(0.04)     | 0.23          | 0.52          | 1.67             |
| M4(1.0)          | C5(1.0)          | none         | 0.08          | 0.20          | 3.06             |
| M4(1.0)          | C5(1.0)          | D1(0.04)     | 0.10          | 0.22          | 1.88             |

\*Weight ratios are in parenthesis.

It is evident from the data in Table IV that the carbonamide coupler solvent C5 substantially reduced the undesirable high delta Dmin values due to continued coupling, both without and with added DIR. It is also evident from the data in Table IV that the use of the carbonamide coupler solvent C5 leads to only slight 55 changes in gamma values relative to those obtained with the conventional solvent S1 for both M3 and M4, either alone or in combination with the inhibitor-releasing coupler D1. That carbonamide C5 reduces continued coupling of M3 and M4, both with and without added inhibitor-releasing coupler D1, is itself surprising. However, even more unexpected and advantageous is that the use of a carbonamide coupler solvent like C5 does not substantially alter gamma values relative to a conventional coupler solvent, even in the presence of a DIR coupler. This is surprising because the carbonamide coupler solvent might have been expected to alter the activity of couplers M3 or M4 relative to the activity of DIR coupler D1, thereby producing undesirably 60 65

large changes in gamma values compared to those obtained with a conventional coupler solvent such as S1. The carbonamides apparently lessen continued coupling by reducing the activity of the two-equivalent pyrazolone couplers at low pH without significantly lowering the activity of the pyrazolone coupler at development pH (10), thereby maintaining a desirable balance between the activities of the pyrazolone coupler and the DIR coupler.

## EXAMPLE 5

Dispersions of the pyrazolone magenta dye-forming couplers M3 and M8, together with S1 and D1 or with C1 and D1, were prepared. These dispersions were coated on a transparent support at a coupler laydown of 0.54 mmole/m<sup>2</sup> together with a silver halide emulsion at a silver laydown of 1.08 g/m<sup>2</sup>, as in Example 2. The coated level of D1 was 0.022 g/m<sup>2</sup>. Coatings were exposed and processed as in Example 2, and the Dmin and gamma values were measured. Table V lists the differences in Dmin values obtained with process B versus process C (a measure of continued coupling) along with gamma values.

TABLE V

| Imaging Coupler | Coupler Solvent* | DIR Coupler* | Delta Dmin Process B - C | Gamma |
|-----------------|------------------|--------------|--------------------------|-------|
| M3(1.0)         | S1(1.0)          | D1(0.040)    | 0.20                     | 1.63  |
| M3(1.0)         | C1(1.0)          | D1(0.040)    | 0.13                     | 1.73  |
| M8(1.0)         | S1(1.0)          | D1(0.043)    | 0.57                     | 2.62  |
| M8(1.0)         | C1(1.0)          | D1(0.043)    | 0.25                     | 1.91  |

\*Weight ratios are in parentheses.

The data in Table V shows the use of C1 in place of S1, with M3 and D1 or with M8 and D1, produces substantial reductions in delta Dmin without greatly altering gamma, that is, without greatly upsetting the balance in reactivity between M3 and D1 or between M8 and D1.

The preceding examples are set forth to illustrate specific embodiments of the invention and are not intended to limit the scope of the materials and methods of the present invention. Additional embodiments and advantages within the scope of the claimed invention will be apparent to one of ordinary skill in the art.

What is claimed is:

1. A color photographic material, comprising a support bearing a silver halide emulsion and a coupler composition comprising (a) a two-equivalent pyrazolone magenta dye-forming coupler, (b) a carbonamide compound of the formula



wherein, R<sub>6</sub>, R<sub>7</sub> and R<sub>8</sub> are individually selected from the group consisting of (i) straight chain, branched and cyclic alkyl groups, straight chain and branched alkenyl groups and straight chain and branched alkylene groups, (ii) said alkyl groups, alkenyl groups and alkylene groups containing one or more substituents selected from the group consisting of alkoxy, aryloxy, aryl, alkoxycarbonyl, aryloxycarbonyl, and acyloxy groups and halogens; (iii) a phenyl group; and (iv) a phenyl group containing one or more substituents selected from the group consisting of alkyl, alkoxy, aryloxy, alkoxycarbonyl, aryloxycarbonyl and acyloxy groups and halogens; and further wherein R<sub>6</sub>, R<sub>7</sub> and R<sub>8</sub> combined

contain at least 12 carbon atoms, and (c) a developer inhibitor-releasing coupler.

2. A color photographic material as defined by claim 1, wherein the two-equivalent pyrazolone magenta dye-forming coupler is of the formula:



wherein:

Ar is selected from the group consisting of unsubstituted aryl groups, substituted aryl groups and substituted pyridyl groups, the substituents being selected from the group consisting of halogen atoms and cyano, alkylsulfonyl, arylsulfonyl, sulfamoyl, sulfonamido, carbamoyl, carbonamido, alkoxy, acyloxy, aryloxy, alkoxy carbonyl, aryloxycarbonyl, ureido, nitro, alkyl and trifluoromethyl groups; Y is selected from the group consisting of anilino, acylamino and ureido groups and one of said groups substituted with one or more substituents selected from the group consisting of halogen atoms, and alkyl, aryl, alkoxy, aryloxy, carbonamido, carbamoyl, sulfonamido, sulfamoyl, alkylsulfonyl, arylsulfonyl, alkylsulfonyl, arylsulfonyl, alkoxycarbonyl, aryloxycarbonyl, acyl, acyloxy, ureido, imido, carbamate, heterocyclic, cyano, trifluoromethyl, alkylthio, nitro, carboxyl and hydroxyl groups, and groups which form a link to a polymeric chain, and wherein Y contains at least 6 carbon atoms; and

X is a coupling-off group selected from the group consisting of halogen atoms, and alkoxy, aryloxy, alkylthio, arylthio, acyloxy, sulfonamido, sulfonyloxy, carbonamido, arylazo, nitrogen-containing heterocyclic and imido groups.

3. A color photographic material as defined by claim 2, wherein Ar is of the formula:



wherein R<sub>1</sub> is selected from the group consisting of halogen atoms and cyano, alkylsulfonyl, arylsulfonyl, sulfamoyl, sulfonamido, carbamoyl, carbonamido, ureido, alkoxycarbonyl, aryloxycarbonyl, acyloxy, alkoxy, aryloxy, nitro and trifluoromethyl groups.

4. A color photographic material as defined by claim 2, wherein Y is of the formula:



wherein

$p$  is from zero to 2 and each  $R_2$  is in a meta or para position with respect to  $R_3$ ; each  $R_2$  is individually selected from the group consisting of halogen atoms and alkyl, alkoxy, aryloxy, carbonamido, carbamoyl, sulfonamido, sulfamoyl, alkylsulfonyl, arylsulfonyl, alkylsulfonyl, arylsulfonyl, alkoxycarbonyl, aryloxycarbonyl, acyloxy, ureido, imido, carbamate, heterocyclic, cyano, nitro, acyl, trifluoromethyl, alkylthio and carboxyl groups, and;

$R_3$  is selected from the group consisting of hydrogen, halogen atoms and alkyl, alkoxy, aryloxy, alkylthio, carbonamido, carbamoyl, sulfonamido, sulfamoyl, alkylsulfonyl, arylsulfonyl, alkoxycarbonyl, acyloxy, acyl, cyano, nitro and trifluoromethyl groups.

5. A color photographic material as defined by claim 2, wherein X is of the formula:



wherein  $R_4$  and  $R_5$  are individually selected from the group consisting of hydrogen, halogen atoms and alkyl, alkoxy, aryloxy, carbonamido, ureido, carbamate, sulfonamido, carbamoyl, sulfamoyl, acyloxy, alkoxycarbonyl, aryloxycarbonyl, amino and carboxyl groups; and wherein  $q$  is 0, 1 or 2 and  $R_5$  may be in the meta or para position with respect to the sulfur atom.

6. A color photographic material as defined by claim 5, wherein  $R_4$  contains at least one carbon atom, and further wherein the total number of carbon atoms in  $R_4$  and  $R_5$  is from about 5 to about 25.

7. A color photographic material as defined by claim 1, wherein  $R_6$ ,  $R_7$  and  $R_8$  combined contain from about 15 to about 30 carbon atoms.

8. A color photographic material as defined by claim 1, wherein at least one of  $R_6$ ,  $R_7$  and  $R_8$  is an alkyl group.

9. A color photographic material as defined by claim 8, wherein  $R_6$ ,  $R_7$  and  $R_8$  individually comprise alkyl groups.

10. A color photographic material as defined by claim 1, wherein  $R_6$  and  $R_7$  or  $R_7$  and  $R_8$  form a ring.

11. A color photographic material as defined by claim 10, wherein  $R_6$  and  $R_7$  or  $R_7$  and  $R_8$  form a five-membered pyrrolidinone ring.

12. A color photographic material as defined by claim 1, wherein the developer inhibitor-releasing coupler includes an inhibitor coupling-off group (IN) selected from the following formulas (VI)–(X):



(VI)



(VII)



(VIII)



(IX)



(X)

25 wherein  $R_9$  is selected from the group consisting of straight and branched alkyls of from 1 to about 8 carbon atoms, benzyl and phenyl groups and said groups containing at least one alkoxy substituent;  $R_{10}$  is selected from  $R_9$  and  $-SR_9$ ;  $R_{11}$  is a straight or branched alkyl group of from 1 to about 5 carbon atoms and  $m$  is from 1 to 3; and  $R_{12}$  is selected from the group consisting of hydrogen, halogens and alkoxy, phenyl and carbonamido groups,  $-COOR_{13}$  and  $-NHCOR_{13}$  wherein  $R_{13}$  is selected from substituted and unsubstituted alkyl and aryl groups.

30 13. A color photographic material as defined by claim 12, wherein the developer inhibitor-releasing coupler includes a timing group which produces a time-delayed release of the inhibitor group and which is selected from the following formulas (XI) and (XII):



(XI)



(XII)

55 60 wherein IN is the inhibitor coupling-off moiety, Z is selected from the group consisting of nitro, cyano, alkylsulfonyl and sulfonamido groups;  $n$  is 0 or 1; and  $R_{14}$  is selected from the group consisting of substituted and unsubstituted alkyl and phenyl groups.

65 14. A color photographic material as defined by claim 1, wherein the carbonamide compound is included in the coupler composition in an amount sufficient to re-

duce continued coupling of the pyrazolone magenta dye-forming coupler during a bleach step in a color photographic process.

15. A color photographic material as defined by claim 1, wherein the coupler composition comprises the pyrazolone magenta dye-forming coupler and the carbonamide compound in a weight ratio of from about 1:0.1 to about 1:10. 5

16. A color photographic material as defined by claim 1, wherein the coupler composition comprises the pyrazolone magenta dye-forming coupler and the developer inhibitor-releasing coupler in a weight ratio of from about 1:0.01 to about 1:2.0. 10

17. A method of forming a color photographic image, comprising (A) imagewise exposing a photographic layer, and (B) developing the exposed image, wherein the photographic layer comprises (a) a two-equivalent pyrazolone magenta dye-forming coupler, and (b) a carbonamide compound of the formula 20



wherein, R<sub>6</sub>, R<sub>7</sub> and R<sub>8</sub> are individually selected from the group consisting of (i) straight chain, branched and cyclic alkyl groups, straight chain and branched alkenyl groups and straight chain and branched alkylene groups, (ii) said alkyl groups, alkenyl groups and alkylene groups containing one or more substituents selected from the group consisting of alkoxy, aryloxy, aryl, alkoxycarbonyl, aryloxycarbonyl, and acyloxy groups and halogens; (iii) a phenyl group; and (iv) a phenyl group containing one or more substituents selected from the group consisting of alkyl, alkoxy, aryloxy, alkoxy carbonyl, aryloxycarbonyl and acyloxy groups and halogens; and further wherein R<sub>6</sub>, R<sub>7</sub> and R<sub>8</sub> combined contain at least 12 carbon atoms, and (c) a developer inhibitor-releasing coupler. 25 30 35

18. A color photographic material, comprising a support bearing a silver halide emulsion and a coupler composition comprising 40

(a) a two-equivalent pyrazolone magenta dye-forming coupler of the formula 45



50

55

wherein:

Ar is selected from the group consisting of unsubstituted aryl groups, substituted aryl groups and substituted pyridyl groups, the substituents being selected from the group consisting of halogen atoms and cyano, alkylsulfonyl, arylsulfonyl, sulfamoyl, sulfonamido, carbamoyl, carbonamido, alkoxy, acyloxy, aryloxy, alkoxy carbonyl, aryloxycarbonyl, ureido, nitro, alkyl and trifluoromethyl groups;

Y is selected from the group consisting of anilino, acylamino and ureido groups and one of said groups substituted with one or more substituents selected from the group consisting of halogen atoms, and alkyl, aryl, alkoxy, aryloxy, carbonamido, carbamoyl, sulfonamido, sulfamoyl, alkylsulfoxyl, arylsulfoxyl, alkylsulfonyl, arylsulfonyl, alkoxy carbonyl, aryloxycarbonyl, acyl, acyloxy, ureido, imido, carbamate, heterocyclic, cyano, trifluoromethyl, alkylthio, nitro, carboxyl and hydroxyl groups, and groups which form a link to a polymeric chain, and wherein Y contains at least 6 carbon atoms; and

X is a coupling-off group selected from the group consisting of halogen atoms, and alkoxy, aryl oxy, alkylthio, arylthio, sulfonamido, sulfonyloxy, carbonamido, arylazo, nitrogen-containing heterocyclic and imido groups,

(b) a carbonamide compound of the formula



wherein, R<sub>6</sub>, R<sub>7</sub> and R<sub>8</sub> are individually selected from the group consisting of (i) straight chain, branched and cyclic alkyl groups, straight chain and branched alkenyl groups and straight chain and branched alkylene groups, (ii) said alkyl groups, alkenyl groups and alkylene groups containing one or more substituents selected from the group consisting of alkoxy, aryloxy, aryl, alkoxycarbonyl, aryloxycarbonyl, and acyloxy groups and halogens; (iii) a phenyl group; and (iv) a phenyl group containing one or more substituents selected from the group consisting of alkyl, alkoxy, aryloxy, alkoxy carbonyl, aryloxycarbonyl and acyloxy groups and halogens; and further wherein R<sub>6</sub>, R<sub>7</sub> and R<sub>8</sub> combined contain at least 12 carbon atoms; and

(c) a developer inhibitor-releasing coupler.

\* \* \* \* \*

60

65